

Patented June 8, 1937

2,083,247

1575  
1575X1526  
X1525

## UNITED STATES PATENT OFFICE

2,083,247

## LUBRICATING OIL

Kenneth Taylor, Chicago, Ill., and Bernard H. Shoemaker, Hammond, Ind., assignors to Standard Oil Company, Chicago, Ill., a corporation of Indiana

No Drawing. Application February 23, 1933,  
Serial No. 658,150

## 1 Claim. (Cl. 196—13)

This invention relates to a method of treating mineral lubricating oils and it pertains more particularly to the art of preparing lubricating oils stable to oxidation and sludging.

5 Petroleum is essentially a mixture of hydrocarbons comprising several groups or homologous series of compounds, such as the paraffins, hydroaromatics, aromatics, polymethylenes, and various other series of compounds in which the hydrogen to carbon ratio varies to a wide degree. A large number of individual compounds of each series are present and have different boiling points, physical and chemical properties. In the various types of crude petroleum commonly 10 known as paraffin base, naphthene or asphalt base, and mixed base oils, these various series of hydrocarbons are present in different proportions. For example, in paraffin base oils, such as those from the Appalachian field, there is a 15 relatively high proportion of paraffinic hydrocarbons having a chain structure and a high hydrogen to carbon ratio, whereas in the California and Gulf Coastal oils there is a high proportion of naphthenic hydrocarbons and hydrocarbons 20 with ring structures and low hydrogen to carbon ratio. The mixed base oils, such as those from Oklahoma and the Mid-Continent area, are in general intermediate between these extreme 25 types.

30 In normal refining of crude petroleum, the fractions of varying distillation ranges which are successively obtained by distillation of the oils partake of the general character of the crude; for example, lubricating oils derived from Appalachian crudes will show paraffinic characteristics, whereas the lubricating oils derived from Gulf Coastal oils show naphthenic characteristics. The distillates from the mixed base crudes, such as those from the Mid-Continent area, will 35 40 show characteristics common to both the naphthenic and paraffinic oils. An important property of paraffinic lubricating oils is their low viscosity temperature coefficient or rate of change of viscosity with temperature. This property makes them particularly suitable for certain lubrication problems where high temperatures are 45 encountered. At low temperatures also, these oils retain their fluidity better, an important consideration in cold weather operation of automobiles, for example. For this reason it is very 50 desirable to separate the mixed base oils into their paraffinic constituents and non-paraffinic constituents.

55 The paraffinic characteristics of an oil may be expressed by its viscosity index. The expression

“viscosity index”, as used herein, refers specifically to the index defined by Dean and Davis in Chemical and Metallurgical Engineering, vol. 36, 1929, page 618. The viscosity index of a lubricating oil is an indication of its composition or type, i. e., whether it is a paraffin base or naphthene base oil. Paraffin base oils are arbitrarily assigned a viscosity index of 100, naphthene base oils are assigned a viscosity index of 0, and mixed base oils lie between these extremes. For example, if an oil shows a viscosity index of about 85 to 90, it is evident that the oil is predominately paraffinic in nature.

5 One of the common ways of increasing the paraffinic content of a lubricating oil is to treat the oil with fuming sulfuric acid. The oil and acid are mixed and agitated in the proportion of about one to two pounds of fuming acid for each gallon of oil. The mixture is then allowed to settle and the acid layer, comprising sulfuric acid and acid sludge, settles to the bottom and is drawn off. The top layer comprises an oil which is high in paraffinic compounds. Also, lubricating oil refined in this way contains a relatively 10 large quantity of sulfonic compounds which must be removed before the oil can be satisfactorily used for most lubricating purposes, and this operation is often expensive and wasteful because of troublesome emulsions which are encountered. The quality of the acid treated lubricating oil 15 can be fairly judged from two of its properties, that is, the viscosity index and stability against sludge formation. The sludge stability is determined by bubbling air at the rate of 10 liters per hour into a 250 cc. sample of oil at 340° F. Samples of 10 grams each are withdrawn at intervals and tested to determine the amount of sludge 20 formed for each 10 grams of oil. When the amount of sludge has increased to 10 mg., the 25 number of hours of oxidation is noted and the sludge stability of the oil is then expressed in 30 hours required to form 10 mg. of sludge per ten grams of oil. The amount of sludge is determined by diluting the 10 gram sample of oil with precipitation naphtha, filtering off the precipitation naphtha insoluble residue, and then washing the filter repeatedly with precipitation naphtha—the residue being sludge.

35 Another method of increasing the paraffinic hydrocarbon content of lubricating oils, as exemplified by the viscosity index, is to extract the oil, preferably a dewaxed oil, with an organic solvent such as chlorinated ethers, sulfur dioxide, chlorohydrins, mixtures of nitro-benzene and acetone, sulfur dioxide, and benzene and the 40 45 50 55

like. These solvents have a preferential solubility for the naphthenic constituents of the oil and are capable of separating a mixed base oil into two major fractions. They are the paraffinic fraction of hydrocarbons and the naphthenic fraction of hydrocarbons. These extraction processes are usually carried out by mixing 2 to 5 parts of solvent with about 1 to 2 parts of oil and then heating and agitating the mixture until substantially complete miscibility is obtained. The mixture is then permitted to cool and stratify. The major portion of the solvent and naphthenic aromatic and aromatic-like compounds and hydrocarbons settle to the bottom and the paraffinic portion of the oil segregates into the top layer and is called the raffinate. The lower layer comprising most of the solvent and naphthenic compounds, is then withdrawn from the raffinate. The raffinate is then heated and treated with steam or an inert gas to remove the small amount of solvent dissolved therein. This treated raffinate is clay-treated and may be given subsequent treatments with sulfuric acid in order to obtain good sludge and color stability. Alternatively, the extraction may be carried out in countercurrent manner by methods well known in the art, in which case it will usually be desirable to work at ordinary temperatures or below.

The object of our invention is provide a method 30 of extracting mineral oils so as to impart good

separate from the highly paraffinic oil. The temperature at which this separation is effected is called the extraction temperature. In this particular example we use an extraction temperature of about 60° F. It should be understood, however, that the extraction temperature may vary with different oils and solvent, but generally the extraction temperature is at least 40° F. below the miscibility temperature. Also, the oil may be cooled step-wise, that is, two or more separations 10 may be made at different temperatures.

The solvent containing aluminum chloride and extract, or bottom layer, is withdrawn from the bottom of the agitator, and then the raffinate is stripped with an inert gas or steam to recover the 15 solvents therefrom. Generally, the stripping is performed at a somewhat elevated temperature.

The raffinate or highly paraffinic fraction of the oil may then be clay treated in the ratio of about 300 to 1000 gallons per ton of clay in order to 20 improve the color of the final product. Fuller's earth, bentonite, Attapulgus clay or other suitable decolorizing clay may be used for this purpose.

The first example of the following table discloses the properties of the above oil when treated 25 in the manner and under the conditions hereinabove set forth. The second example discloses the properties of the oil when extracted and treated under the same conditions but in the absence of aluminum chloride.

Table I

| 35 | Example | True color<br>after extrac-<br>tion | Yield<br>(per<br>cent) | Clay<br>treated<br>(gals. per<br>ton) | Saybolt<br>viscosity |         | True<br>color | Viscosity<br>index | Sludging time—<br>hours |         | 35 |
|----|---------|-------------------------------------|------------------------|---------------------------------------|----------------------|---------|---------------|--------------------|-------------------------|---------|----|
|    |         |                                     |                        |                                       | 210° F.              | 100° F. |               |                    | 10 mg.                  | 100 mg. |    |
|    |         |                                     |                        |                                       |                      |         |               |                    |                         |         |    |
| 40 | 1-----  | 136                                 | 69                     | 333                                   | 87                   | 1044    | 3             | 88.5               | 94                      | 129     | 40 |
|    | 2-----  | 256                                 | 67                     | 333                                   | 89                   | 1087    | 13            | 88.5               | 72                      | 112     |    |

sludge and color stability thereto simultaneously with the step of solvent extraction. We have found that a small amount of metal halides such as aluminum chloride dissolved and/or colloidally suspended in the solvent will greatly improve the color and increase the sludge stability of the raffinate.

We will describe our process by extracting a Mid-Continent mixed-base lubricating oil with a single organic solvent containing about 1% of aluminum chloride dissolved and/or suspended therein. In this particular example we will use a Mid-Continent lubricating oil distillate having a Saybolt viscosity of 114 at 210° F. and 2350 at 50 100° F. and a viscosity index of 56.5, sludging time of less than 10 hours for 10 mg. of sludge. However, it should be understood that our process is applicable to any distillate or bottom derived from mixed base oils or naphthenic oils. One 55 volume of the oil is mixed in a suitable agitator with 1.5 volumes of beta-beta' dichlorethyl ether containing about 1% of aluminum chloride. The mixture is then agitated and heated to a temperature somewhat above the miscibility temperature 60 which is about 140° F. In this particular example the mixture was heated to 180° F. Generally the solvent or solvents are miscible with the oil within the range of 50 to 220° F. However, with some solvents the miscibility temperature may be 65 lower than this.

After the oil and solvent containing aluminum chloride have been heated to the miscibility temperature, the mixture is cooled to a temperature below the miscibility temperature where the solvent 70 containing aluminum chloride and extract

From Example 2 of the above table, which gives the results of the extraction in the absence of aluminum chloride, it will be noted that the true color of the raffinate before claying was 256; after claying the true color was 13. The time required for 10 mg. of sludge to form under the excessive oxidizing conditions was 72 hrs. and the time required for 100 mg. of sludge to form was 112 hours. Example 1 discloses the properties of the oil when treated under exactly the same conditions but in the presence of 1% by weight of aluminum chloride. It will be observed that the true color of the raffinate after this extraction was 136; after claying the true color was 3—a great improvement over the color obtained in the absence of aluminum chloride. The time required for 10 mg. of sludge to form was 94 hrs. and the time required for 100 mg. of sludge to form was 129 hrs.

In view of the above table and explanation it is apparent that the presence of a small amount of aluminum chloride in the solvent greatly decreases the true color and adds increased sludge stability to the oil. It should be observed that there is no decrease in the yield or viscosity index of the oil in order to obtain this improved color and sludge stability. In fact, it will be noted that a slight increase in yield was obtained. If the above oil is treated with aluminum chloride per se, about 9%, the sludge stability is very low. In fact, it required only 31 hrs. to form 10 mg. of sludge.

The following table sets forth the properties of the refined oil obtained by the hereinbefore described process when one volume of distillate 75

(114 Saybolt viscosity at 210° F., 2350 Saybolt viscosity at 100° F. and a viscosity index of 56.5) is extracted with one volume of the halogenated ether in the presence of 2% of aluminum chloride by weight at 160° F.

Table II

| 10 | True color after extraction | Yield (per cent) | Clay treated (gals. per ton) | Saybolt viscosity |         | True color | Viscosity index |
|----|-----------------------------|------------------|------------------------------|-------------------|---------|------------|-----------------|
|    |                             |                  |                              | 210° F.           | 100° F. |            |                 |
|    | 82                          | 78               | 1000                         | 93.2              | 1286    | 13         | 81              |

15 By comparing the properties of the oil set forth in Table II with the properties of the oil in Example 2 of Table I it will be observed that the true color of the oil after claying are the same, but 1000 gals. of oil were treated per ton of clay in the case of the oil in Table II and only 333 gals. were treated per ton of clay in the case of the oil in Example 2 of Table I. It will be noted that the extraction with a solvent in the presence of a small amount of aluminum chloride provides a process of obtaining 1000 gals. of oil of 13 true color per ton of clay, whereas, in the absence of aluminum chloride only 333 gals. of oil of 13 true color were obtained per ton of clay.

30 The second example of the following table represents the results obtained when one volume of the above oil (Saybolt viscosity of 114 at 210° F., 2350 at 100° F. and a viscosity index of 56.5) is treated with 1½ volumes of nitrobenzene containing 1% by weight of aluminum chloride. The treating temperature used in this example was 200° F. The first example of this table discloses the properties of the above oil when treated under the same conditions with the same solvent but in the absence of aluminum chloride.

Table III

| 45 | Example | True color after extraction | Yield (per cent) | Clay treated (gals. per ton) | Saybolt viscosity |         | True color | Viscosity index | Sludging time—hours |         |
|----|---------|-----------------------------|------------------|------------------------------|-------------------|---------|------------|-----------------|---------------------|---------|
|    |         |                             |                  |                              | 210° F.           | 100° F. |            |                 | 0 mg.               | 100 mg. |
| 1  |         | 90                          | 62               | 1,000                        | 87.8              | 1111    | 39         | 84              | 39                  | 69      |
| 2  |         | 64                          | 62               | 1,000                        | 87.8              | 1094    | 13         | 85.5            | 67                  | 114     |

55 From Example 2 of the above table it will be observed that the color and sludge stability of the oil treated in the presence of aluminum chloride is greatly improved. It is apparent that the presence of a small amount of aluminum chloride materially decreases the true color of the oil and adds increased sludge stability to the oil. Furthermore, it will be observed that 60 these enhanced properties were obtained without the loss of yield or viscosity index. In fact, the viscosity index of the oil which was treated with nitrobenzene containing aluminum chloride dissolvent and/or dispersed therein was slightly better than the oil which was extracted with the same solvent but in the absence of aluminum chloride. White oils, or substantially colorless mineral oils can be prepared by our process by repeating the extraction of the oil 65 several times with the solvent and metallic halide. The degree of refining will determine the number of extractions. Petroleum naphthas may likewise be refined by our process as hereinbefore described.

70 Instead of using the hereinabove mentioned

solvents in the presence of metallic halides, we may use other organic selective solvents. Examples of solvents which may be used in combination with these metallic chlorides such as aluminum chloride, boron trichloride and zinc chloride are: methyl 2-chloorethyl ether, di(2-chloorethyl)ether, methyl chloropropyl ether, methyl 2-3 dichloropropyl ether, ethyl 2-3 dichloropropyl ether, 2-chloorethyl ether, dichlorisopropyl ether, dichloropropyl ether, nitrobenzene, nitrotoluene, nitroxylene, ethyl chloracetate, ethyl dichloracetate, ethyl chloropropionate, 2-chloorethyl acetate, methyl chloracetate, 2-chloorethyl propionate, sulfur dioxide, dioxane, pyridine, nitronaphthalene, or mixtures of the above. We have found that the alpha chlorinated aliphatic ethers and esters are more reactive than the beta or gamma halogenated compounds and that satisfactory results are not obtained with these alpha halogenated compounds.

75 Instead of using a single organic solvent in the presence of these metallic halides, we may use mixed solvents in combination with aluminum chloride, boron tri-chloride or zinc chloride. Examples of mixed solvents which may be used for extracting lubricating oils are:

Table IV

|                                                 |    |
|-------------------------------------------------|----|
| Acetone and nitrobenzene                        | 30 |
| Acetone and di(2-chloorethyl)ether              |    |
| Acetone and dichlorobenzene                     |    |
| Acetone and cresol                              |    |
| Methyl ethyl ketone and di(2-chloorethyl)ether  |    |
| Methyl propyl ketone and nitrobenzene           | 35 |
| Methyl propyl ketone and di(2-chloorethyl)ether |    |
| Ethyl acetate and nitrobenzene                  |    |
| Ethyl acetate and di(2-chloorethyl)ether        |    |
| Carbon dioxide and sulfur dioxide               |    |
| Propyl ether and nitrobenzene                   | 40 |
| Iso-propyl ether and nitrobenzene               |    |

50 Iso-propyl ether and chlorinated aliphatic ethers  
Methyl acetate and nitrobenzene  
Methyl acetate and di(2-chloorethyl)ether  
Propyl acetate and nitrobenzene  
Ethyl propionate and nitrobenzene  
Ethyl propionate and di(2-chloorethyl)ether  
Methyl propionate and nitrobenzene  
Sulfur dioxide and benzene  
Sulfur dioxide and dimethyl ether  
Sulfur dioxide and diethyl ether

55 The metallic halides which have proven most desirable for this process are substantially anhydrous aluminum and zinc chloride, ferric chloride, magnesium chloride, and boron tri-chloride and fluoride. The commercial grades of these reagents are satisfactory. The amount used may vary from 0.5 to 3%, or even up to 10%, but generally 1% is adequate.

60 The proportions of the above solvents used to extract the oil may vary under different conditions, but generally these extractions are carried out by mixing one to five parts of the solvent with about 0.5 to one part of oil.

65 The term "naphthenic hydrocarbons" is em-

ployed in this specification and claim in a generic sense to include the compounds that have a low viscosity index, low A. P. I. gravity, and usually rapid sludge-forming characteristics, examples of which are the aromatic, aromatic-like, olefins, high molecular weight polymethylenes, nitrogen and sulfur compounds.

The term "non-sludging" and "stable to oxidation and sludging" is used in the specification and claim to cover an oil which has greater sludge stability than the parent oil. These terms are not intended to define oils that are absolutely stable against sludge formation under rigid oxidizing conditions for long periods of time.

In addition to or instead of extracting the lubricating oils in the presence of aluminum chloride, we may first treat the oil with aluminum chloride and then extract with a selective solvent. However, this procedure is usually more expensive for the reason that it requires additional operations after the extraction with the solvent. We have found that the process of extracting in the presence of aluminum chloride is very economical.

The oil treated by our process may be dewaxed

before and/or after the extraction, but we prefer to dewax the oil before extraction. While we have described our invention with reference to specific materials and proportions of solvents, it should be understood that the scope of our invention is not limited thereto except insofar as set forth in the appended claim.

We claim:

The method of preparing a non-sludging lubricating oil having a low true color from a mineral oil containing naphthenic and paraffinic constituents, the steps comprising mixing one volume of said mineral oil with at least one volume of a selective solvent selected from the group consisting of di(2-chlorethyl)ether and nitrobenzene which has a small amount of aluminum chloride dissolved therein, heating said mixture to an elevated temperature to effect substantially complete solution, cooling said admixture to a temperature at which phase separation occurs, withdrawing the top layer and removing therefrom the dissolved solvent.

KENNETH TAYLOR.  
BERNARD H. SHOEMAKER.